

# United States Patent Office

2,879,195

Patented Mar. 24, 1959

1

2,879,195

## FLUX

David B. Speed, Cleveland, Ohio, and Ivan R. Smith, North Augusta, S.C., assignors to E. I. du Pont de Nemours and Company, Wilmington, Del., a corporation of Delaware

No Drawing. Application August 31, 1956  
Serial No. 607,254

8 Claims. (Cl. 148—23)

This invention relates to galvanizing fluxes and is more particularly directed to compositions adapted to be used in a flux wash and comprising, preferably, zinc ammonium chloride and an alkyl sulfonate.

It is customary to prepare metals prior to galvanizing and prior to introduction into a molten metal bath by passing them through an aqueous solution which is called a "flux wash." Such solutions customarily contain fluxing materials such as zinc chloride, ammonium chloride, and zinc ammonium chloride.

It is important, especially in some of the new high-speed continuous galvanizing processes, that the flux wash thoroughly wet the surface of the metal and yet the solution must not foam excessively. If there is any considerable foaming in the flux wash, the high speeds at which the metal is traveling cause an excessive "drag-out" from the flux wash bath.

We have found that improved flux wash compositions can be prepared from ammonium chloride, zinc chloride, zinc ammonium chloride, and other such reflux compositions by the addition thereto of an alkyl sulfonate.

Most preferred for flux wash compositions of the invention are the so-called "high ratio" zinc ammonium chlorides. These are flux compositions in which the weight ratio of  $ZnCl_2:NH_4Cl$  ranges from 1.27:1 to 1.35:1. These are normally made up into prewash fluxes of about 12.2° Baumé strength and used at temperatures around 180° F.

The prewash flux compositions of the invention are made up by the addition to one of the flux materials described, and preferably to a high ratio zinc ammonium chloride, of a small amount of an alkyl sulfonate. The alkyl sulfonate has the formula:



in which R is a higher alkyl group ranging from about 8 to 18 carbon atoms.

The commercially available material which is preferred contains minor amounts of sodium sulfate and sodium chloride and R is approximately  $C_{13}$ , which corresponds to the kerosene fraction. The  $SO_3Na$  groups are randomly distributed.

The alkyl sulfonate is prepared as a solution in water and is sprayed onto the flux material, say, zinc ammonium chloride, in the form of dry crystals. This is done while the zinc ammonium chloride crystals are tumbled to obtain even distribution of the alkyl sulfonate.

The amount of the alkyl sulfonate to be used with various flux materials can be widely varied, though generally only as much will be used as is required to obtain a desired effect. Broadly, there can be used from about 0.04 to 0.4 gram of alkyl sulfonate per 100 grams of zinc ammonium chloride or of the other fluxes mentioned. More narrowly, from about 0.04 to 0.13 gram of alkyl sulfonate is preferred per 100 grams of flux material such as zinc ammonium chloride.

In order that the invention may be better understood,

2

reference should be had to the following illustrative examples.

### Example 1

A 10% aqueous solution was prepared of an alkyl sulfonate. The alkyl sulfonate contained sulfonates of the formula  $R-SO_3Na$  in which the  $SO_3Na$  groups were randomly distributed and in which R approximates  $C_{13}$  (kerosene). The product contained minor amounts of sodium sulfate and sodium chloride as well as a small amount of unreacted alkane.

The aqueous solution thus prepared was sprayed onto zinc ammonium chloride having a  $ZnCl_2:NH_4Cl$  ratio of 1.3:1.

The amount of the alkyl sulfonate based upon the zinc ammonium chloride was about 0.1 gram of alkyl sulfonate for each 100 grams of zinc ammonium chloride.

The dry product thus obtained was formed into a flux wash by dissolving in water to form a 12.2° Baumé solution which contained about 24.5 percent by weight of zinc ammonium chloride.

Instead of using high ratio zinc ammonium chloride as above described, compositions adapted for the preparation of flux washes can be made up by using an alkyl sulfonate at the rates as above described with zinc chloride, with ammonium chloride, or with low ratio zinc ammonium chloride.

### Example 2

A 22% aqueous solution of an alkyl sulfonate was prepared as in Example 1. This was sprayed onto zinc ammonium chloride as in Example 1 using 0.41 gram of the solution for each 100 grams of zinc ammonium chloride.

The dry product thus obtained was used as a flux wash and even lower foaming was obtained than with the flux wash of Example 1.

Instead of using the high ratio zinc ammonium chloride, there can be used zinc chloride, ammonium chloride, or a low zinc ammonium chloride.

This application is a continuation-in-part of our pending application Serial No. 539,263, filed October 7, 1955, now abandoned.

We claim:

1. A galvanizing flux consisting essentially of a fluxing material selected from the group consisting of ammonium chloride, zinc chloride, and zinc ammonium chloride and 0.04 to 0.4 gram of an alkyl sulfonate per 100 grams of said fluxing material.

2. A dry galvanizing flux consisting essentially of zinc ammonium chloride and 0.04 to 0.13 gram of an alkyl sulfonate per 100 grams of zinc ammonium chloride.

3. A dry galvanizing flux consisting essentially of zinc ammonium chloride with a  $ZnCl_2:NH_4Cl$  weight ratio of 1.27:1 to 1.35:1 and 0.04 to 0.4 gram per 100 grams of zinc ammonium chloride of a sodium salt of an alkyl sulfonate in which the alkyl groups average about 13 carbon atoms.

4. A flux wash for application to metals prior to galvanizing consisting essentially of an aqueous bath containing zinc ammonium chloride and 0.04 to 0.4 gram per 100 grams of zinc ammonium chloride of an alkyl sulfonate.

5. A dry galvanizing flux composition for use as a high-speed continuous galvanizing flux wash consisting essentially of zinc ammonium chloride with a



weight ratio of from about 1.27:1 to 1.35:1 and from about 0.04 to 0.13 gram per 100 grams of zinc ammonium chloride of a sodium salt of an alkyl sulfonate in which the alkyl groups average about 13 carbon atoms.

6. A dry galvanizing flux composition for use as a high-speed continuous galvanizing flux wash consisting essentially of zinc ammonium chloride with a



weight ratio of from about 1.27:1 to 1.35:1 and from about 0.04 to 0.13 gram per 100 grams of zinc ammonium chloride of a sodium salt of an alkyl sulfonate in which the alkyl groups average about 13 carbon atoms, each such composition containing the alkyl sulfonate coated upon the zinc ammonium chloride. 10

7. A method for the preparation of a high-speed galvanizing flux composition comprising spraying an aqueous solution of an alkyl sulfonate onto zinc ammonium chloride crystals, such crystals being tumbled to obtain even 15 distribution of the alkyl sulfonate, the spraying being continued until from about 0.04 to 0.4 gram of alkyl sulfonate have been applied to each 100 grams of zinc ammonium chloride.

5

8. A method for the preparation of a high-speed galvanizing flux composition comprising spraying upon tumbled dry crystals of zinc ammonium chloride an aqueous solution of an alkyl sulfonate in which the alkyl groups preferably each average about 13 carbon atoms until from about 0.04 to 0.4 gram of such alkyl sulfonate have been applied to each 100 grams of said zinc ammonium chloride.

References Cited in the file of this patent

UNITED STATES PATENTS

|           |               |                |
|-----------|---------------|----------------|
| 1,965,759 | Baldwin       | July 10, 1934  |
| 2,174,507 | Tinker et al. | Sept. 26, 1939 |
| 2,311,669 | Kepfer        | Feb. 23, 1943  |
| 2,327,958 | Carey         | Aug. 24, 1943  |
| 2,508,501 | Di Giulio     | May 23, 1950   |

UNITED STATES PATENT OFFICE  
CERTIFICATE OF CORRECTION

Patent No. 2,879,195

March 24, 1959

David B. Speed et al.

It is hereby certified that error appears in the printed specification of the above numbered patent requiring correction and that the said Letters Patent should read as corrected below.

Column 2, line 38, after "low" insert — ratio —.

Signed and sealed this 8th day of September 1959.

(SEAL)

Attest:

KARL H. AXLINE

Attesting Officer

ROBERT C. WATSON  
Commissioner of Patents